# EUROPEAN PATENT SPECIFICATION

(11) **EP 1 299 509 B1**
(45) Date of publication and mention of the grant of the patent: **25.08.2004**
(21) Application number: 01949345.1
(22) Date of filing: 17.05.2001
(51) Int. Cl.: C10M 141/06

(54) **FRICTION MODIFIER ADDITIVE COMBINATION**
REIBUNGSMODIFIZIERENDE ZUSATZKOMBINATION
MELANGE D'ADDITIFS A FONCTION DE MODIFICATEUR DE FROTTEMENT

(30) Priority: 17.05.2000 GB 0011931
(43) Date of publication of application: 09.04.2003
(73) Proprietor: ExxonMobil Research and Engineering Company, Annandale, New Jersey 08801 (US)
(72) Inventor: STEIGERWALD, Edgar, Andreas, Hamburg (DE)
(74) Representative: Troch, Geneviève
(86) International application number: PCT/EP2001/005656
(87) International publication number: WO 2001/088067

(56) References cited:
- EP-A- 0 747 464
- EP-A- 0 748 862
- EP-A- 0 812 900
- WO-A-93/06198
- WO-A-97/04049
- WO-A-97/09401
- WO-A-98/39400
- WO-A-99/02628
- US-A- 5 646 099
- US-A- 5 773 393

## Description

This invention relates to a combination of additives that provides friction modifier benefits to lubricants and functional fluids, especially to power transmission fluids such as gear oils, automatic transmission fluids and fluids for continually variable transmissions.

Power transmissions for automotive vehicles, for example automatic transmissions, are being continually developed to improve their performance. There is a new generation of automatic transmissions currently being produced which are equipped with an electronically controlled converter clutch (hereafter "ec³"). The design provides a more compact and lighter automatic transmission that enables together with the ec³ a fuel saving of up to 10% and exhibits superior shift comfort.

The new automatic transmission designs place higher demands on the automatic transmission fluid (hereafter "ATF"). All ATFs should possess high oxidation stability, good viscometrics and low temperature properties, as well as good corrosion protection, anti-foaming and air separation properties. In addition, the friction properties, measured by friction coefficients displayed in a graph, are key to providing satisfactory performance. The friction property of the ATF must be balanced such that there is sufficient friction to provide adequate power transmission whilst minimising shudder both on start up of the engine (the so called "green shudder") and over the lifetime of the ATF. Excessive shudder causes driver discomfort and gives rise to an unacceptable noise level.

For the recently developed automatic transmissions equipped with an electronically controlled converter clutch, these friction requirements are even more demanding. Typically, the Original Equipment Manufacturer (hereafter "OEM") specifies a minimum friction coefficient at a plate sliding speed of 5 rpm of 0.123 to provide the necessary power transmission to the axle, together with the requirement that the friction coefficient does not decrease with increasing plate sliding speed, ie the gradient of the curve in the graph of friction coefficient against increasing sliding speed is positive or zero; it must not be negative. The latter requirements *is* to minimise green shudder to an acceptable time period of no more than 0.2 hours (12 minutes). Furthermore, it is preferred that the ATF will function without noticeable shudder (once any green shudder has ceased) for at least 150,000 km o f automotive transmission operation. The minimum hours according to the Zahnradfarbik Friedrichschafen (hereafter "ZF") ec3 test as defined is in the region of >100 hours.

ATFs used hitherto containing conventional friction modifiers (hereafter "FM"), such as fatty acids, fatty amines and fatty alcohols, do not meet these requirements. For example, ETHOMEEN® T-12, a tallow amine supplied by AKZO Chemicals, when incorporated in an ATF formulation at a treat level of 0.15% by wt. does not always meet the requirement for friction coefficient vs. sliding speed (0.123 at 5 rpm) and never achieves a durability of >100 hours.

Prior published EP-A-0 713 908 describes an oil-based power transmission fluid composition, especially ATFs which contains *inter alia* at least one oil-soluble friction modifier which may be selected from aliphatic amines, aliphatic fatty acid amides, aliphatic carboxylic acids, aliphatic carboxylic esters, aliphatic carboxylic ester amides, aliphatic phosphonates, aliphatic phosphates, aliphatic thiophosphates and aliphatic thiophosphates etc wherein the aliphatic group contains more than 8 carbon atoms to render the compound suitably oil soluble. The compositions of this invention are said to have the capability of exhibiting a positive slope in the plot of coefficient of friction versus sliding speed in the low speed SAE No. 2 Friction Test when performed with Ford Engineering Material Specification WSP-M2CZAA-A. Also, in clutch friction durability tests performed using the above method involving 20,000 cycles, the following results were achieved: µD in the range of 0.130-0.170; µS values (at 0.25 seconds) in the range of 0.110-0.155; low speed dynamic friction values in the range of 0.130-0.170; S1/D values in the range of 0.90-1.16; and stop times, in seconds, in the range of 0.70-1.0. It would be evident to those skilled in the art that this SAE-test cannot be read across for European OEMs, and hence it is not suitable for European design because it is a laboratory test rig which did not produce the specific results initially and, therefore, had to be abandoned.

WO 99/02628 discloses friction modifiers including alkoxylated amines and a polyamide compound which is the reaction product of a polyamine containing from 2 to 60 total carbon atoms and from 3 to 15 nitrogen atoms with at least one of the nitrogen atoms present in the form of a primary amine group and at least two of the remaining nitrogen atoms present in the form of primary or secondary amine group and a carboxylic anhydride.

EP 0748862 relates to lubrication composition, that may be used as automatic or manual transmission fluid, comprising a major amount of an oil of lubricating viscosity and at least one metal free thiophosphorus acid ester, at least one amine salt of the thiophosphorus acid ester, or a mixture thereof, wherein the metal free thiophosphorus acid ester contains at least one hydrocarbyl terminated oxyalkylene group, at least one hydrocarbyl terminated polyoxyalkylene group, or a mixture thereof. EP 812900 discloses a lubricating oil composition for automatic transmission comprising a sulfur-containing antioxidant or an amine type antioxidant, a phosphate or its amine salt and a reaction product of a carboxylic acid and an amine wherein the amine type antioxidant is chosen from alkylarylamines. WO 97/04049 discloses a friction modifier including an alkoxylated amine and a polyamide which is the reaction product of a carboxylic acids or anhydride with a polyamine containing from 2 to 60 total carbon atoms and from 3 to 15 nitrogen atoms with at least one of the nitrogen atom present in the form of a primary amine group and at least two of the remaining nitrogen atoms present in the form of primary or secondary amine groups.

The present invention provides a friction modifier additive combination comprising (a) an oil-soluble fatty amine compound and (b) an oil-soluble fatty amide compound.

It has been found that by combining a fatty amine with a fatty amide, the friction properties of a lubricant or functional fluid containing the same are improved. For example, by formulating an ATF using the amine/amide friction modifier combination of the present invention it is possible to achieve a friction coefficient at 5 rpm of at least 0.123 together with a positive or zero gradient in the graph of friction coefficient versus sliding speed. After the end of the green shudder, if any, the ATF can operate for 150 hours or more before the onset of shudder.

The fatty amine compound is a tertiary amine compound, of formula (I) below: wherein:
R is an alkyl group containing from 8 to 24 carbon atoms or any aryl group containing one or more alkyl substituents containing from 8 to 24 carbon atoms;
R¹ and R² are each independently an alkylene group containing from 1-8 carbon atoms; and x and y are each independently 0 or an integer from 1 to 5.

The substituent group R is suitably an alkyl group containing from 10 to 18 carbon atoms, preferably from 12 to 14 carbon atoms. The substituent group R is suitably derived from a fatty acid which is usually a naturally occurring substance and therefore may contain a mixture of carbon chain lengths, in which case the average chain length of the substituent group R is more preferably within the carbon atom ranges specified above.

The substituent groups R¹ and R² are each independently an alkylene group as stated above and these groups suitably have 1 to 4 carbon atoms, most preferably 2 carbon atoms such as eg a -CH₂-CH₂- grouping. The groupings -R¹O- and -R²O- are preferably oxyethylene groups and correspondingly -R¹OH and -R²OH are ethylenehydroxy groups.

The number of oxyalkylene groups represented by x and y are each independently suitably 0, 1 or 2 and are preferably 0.

Specific examples of suitable fatty amine compounds include a coco-bis(2-hydroxyethyl)amine, a polyoxyethylene(5)coco-amine, a tallow-bis(2-hydroxyethyl)amine, a polyoxyethylene(5)tallow amine, a tallow/oleyl-bis(2-hydroxyethyl)amaine and an oleyl-bis- (2-hydroxyethyl)amine. Such compounds are commercially available from eg AKZO Chemicals. Particularly preferred are compounds such as eg the coco-bis(2-hydroxyethyl)amine (ETOMEEN® C/12) which contains a mixture of C₈ to C₁₈ alkyl groups, with C₁₂ groups predominating sold by Akzo Chemicals.

The fatty amide compound is a tertiary amide of the formula (II) wherein R, R¹, R², x and y are each independently as defined above for formula (I), both in respect of general and preferred embodiments.

Specific examples of suitable fatty amide compounds include the compound polyoxyethylene(5)oleamide sold under the trade name ETHOMID® 0/15 (ex Akzo Chemicals) which contains a mixture of C₁₂ to C₁₈ alkyl groups predominating in C₁₈ groups; and a fatty acid amide derived from lauric acid sold as COMPERLAN® LD (ex Henkel).

In a preferred embodiment, the friction modifier additive combination according to the present invention comprises a mixture of (a) a bis(hydroxyethyl) fatty amine wherein the fatty group comprises an alkyl group which has 12 to 14 carbon atoms and (b) a bis(hydroxyethyl) fatty amide wherein the fatty group comprises an alkyl group which has 12 to 18 carbon atoms.

In another embodiment, the present invention provides a lubricant or functional fluid formulation comprising a major amount of base oil of lubricating viscosity and a minor amount of a friction modifier additive combination as defined above. The lubricant or functional fluid is suitably useable as a power transmission fluid, preferably as an automatic transmission fluid (ATF). To illustrate the invention, the following description will focus on ATF formulations although it will be understood that the compositions of the present invention are not limited to such fluids but embraces within its scope other lubricant and functional fluids.

ATFs typically have a kinematic viscosity at 100°C (KV₁₀₀) ranging from 2-15 mm²/s, preferably from 4-10 mm²/s, more preferably from 5-8 mm²/s measured according to the standard test procedure of ASTM D-446. The Brookfield viscosity at - 40°C is suitably less than 50,000 mPa s, preferably from 4,000-20,000 mPa s, and more preferably from 5,000-18,000 mPa s measured according to the standard test procedure of ASTM D-2983. The viscosity index is suitably in the range from 100-200, preferably from 150-200 measured according to the standard test procedure of ASTM D-2270.

Generally, the amount of base oil contained in the ATF ranges from 50% by weight to 99.9%, suitably from 60-95% by weight and preferably from 70-90% by wt, based on the total weight of the ATF formulation.

The amount of friction modifier additive combination present in the ATF formulation (ie the total amount of fatty amine and fatty amide) is broadly in the range from 0.05-1.2% by weight. Within this range the specific amount used will depend not only upon the friction properties desired but also, at least to some extent, upon the design of the automatic transmission. Thus the amount of friction modifier additive combination used is suitably in the range from 0.1-1% by weight, preferably from 0.2-0.8% by weight and more preferably from 0.3-0.6% by weight.

The amount of fatty amine compound in this friction modifier additive combination is suitably in the range from 0.03-1.0% by weight, preferably from 0.05-0.8% by weight and more preferably from 0.1-0.6% by weight. The fatty amide compound in the additive combination is suitably from 0.05-0.8% by weight, preferably from 0.05-0.5% by weight and more preferably from 0.08-0.3% by weight.

The weight ratio of the fatty amine to fatty amide in the additive combination is suitably in the range from 0.5:1 to 10:1, preferably from 1:1 to 8:1 and more preferably from 2:1 to 6:1.

The amounts of the fatty amine and fatty amide in the additive combination are with respect to the active ingredients in such compounds. The compounds specified above are generally liquids at room temperature and within conventional lubricant additive handling and blending temperatures, and are therefore usually supplied and used in neat, 100% active ingredient form. However, if desired, they may be diluted with a solvent, such as eg mineral oil, which is inert under the conditions especially with respect to the performance of the lubricant.

The base oil of the ATF or other lubricant or functional fluid according to the invention may be a mineral oil, a synthetic oil or mixtures thereof. The base oils are suitably selected from refined mineral oils, for example, a solvent refined and/or hydrotreated oils, oils derived from coal tar or shale, vegetable oils, animal oils, hydrocracked oils, hydroisomerised oils, poly-alphaolefins (PAO), esters, alkylbenzenes, polyglycols, alkylene oxide polymers, silicone oils and the like.

Where the base oil comprises a mineral oil, it is suitably a solvent refined and/or hydrotreated oil. Examples of suitable oils of this type include *inter alia* solvent refined mineral oils in the range of 50N to 150N, preferably 80N to 130N. Such mineral oils are available, for example, from Esso under the trade name Esso Solvent Neutral.

Where the base oil is a severely refined mineral oil such as eg white oil, these may be one of the varieties supplied by Esso under the trade names MARCOL® 52 and 172, PRIMOL® 352, PLASTOL® 135 and 352, and BAYOL® 52. The base oils used may also be a hydrocracked or hydroisomerised oils such as eg a hydroisomerised paraffin.

Where the base oil is a synthetic oil, it is preferably a PAO produced by the oligomerisation of 1-alkenes which suitably contain 6-20 carbon atoms, preferably 8-14 carbon atoms. PAOs produced from 1-decene are particularly preferred. The KV₁₀₀ of the PAO selected is usually determined by the viscosity desired in the final lubricant formulation and is suitably in the range from 2-8mm²/s, preferably from 4-6mm²/s. Such PAOs are commercially available eg from ExxonMobil.

In a preferred embodiment, the base oil is a mix of mineral oils and synthetic oils, eg a mixture of one or more solvent refined mineral oils with PAOs; or a mixture of solvent refined mineral oil with white oil, a hydrocracked oil or a hydroisomerised oil as stated above. In a particularly preferred embodiment, the base oil is a mixture of solvent refined mineral oil, a PAO and white oil.

The functional fluid formulations of the present invention may also contain other optional additives depending upon the intended use of the functional fluid. Such additives include *inter alia* viscosity index improvers, pour point depressants, antioxidants, anti-wear agents, extreme pressure additives, dispersants, detergents, corrosion inhibitors, erosion inhibitors, anti-foaming agents, seal swell conditioning agents (seal fix), anti-pitting agents and the like. Such additives are all commercially available, the choice of one or more of these and the amounts of each used depending upon the intended end use of the functional fluid. Thus, eg, a viscosity index improver would typically be included in the functional fluids at a treat level of 2-15% by weight based on active ingredient (ie excluding solvent and carrier fluids, if any), preferably from 2-10% by weight, and the other additives would typically be included in the functional fluids at a treat level of 0.01-5% by weight based on active ingredient.

The optional additives recited above may be added individually to the base oil, or, two or more may be pre-mixed with a carrier fluid such as eg a mineral oil, to form an additive concentrate and can then be blended with the base oil. The friction modifier additive combination according to the invention may also be pre-mixed with or without other additives into an additive concentrate.

Of the optional additives recited above:
the dispersants are suitably ashless dispersants such as eg polyalkenyl succinic anhydrides, polyalkenyl succinimides and derivatives thereof wherein the polyalkenyl group is derived from a long chain polyolefm such as eg polyisobutylene;
the extreme pressure additives are suitably phosphorus- or zinc-based;
the antioxidants are suitably aminic and/or phenolic type;
the pitting booster is suitably sulphurised fatty oil eg Sulperm® 307 (ex Ferro Corporation);
the anti-foam agents are suitably silicon based; and
the viscosity index improver is suitably acrylic based such as eg a polymethylmethacrylate.

The friction modifier additive combination and lubricating oil formulations produced therefrom are particularly effective when used in automatic transmission fluids, especially for automatic transmissions equipped with an electronically controlled converter clutch.

The present invention is further illustrated with reference to the following Examples.

The following formulation was tested for its performance as an ATF in which all the amounts in the columns are % by weight:

**TABLE 1**

| COMPONENTS | Test No. 1 | Test No. 2 | Test No. 3 | Test No. 4 |
|---|---|---|---|---|
| Mineral base oil (SN90) | 10.0 | 10.0 | 10.0 | 10.0 |
| White oil (Hydrovis® 3) | 30.0 | 30.0 | 30.0 | 30.0 |
| PAO 4 | 30.0 | 30.0 | 30.0 | 30.0 |
| Hydrocracked base oil (Nexbase 3030) | 14.87 | 14.89 | 14.67 | 14.77 |
| X-9077* | 5.6 | 5.6 | 5.6 | 5.6 |
| Pitting booster (Sulperm® 307) | 0.4 | 0.4 | 0.4 | 0.4 |
| Pour point depressant (Viscoplex® 1-311) | 0.2 | 0.2 | 0.2 | 0.2 |
| VI Improver (Viscoplex® 0-030) | 8.5 | 8.5 | 8.5 | 8.5 |
| Parabar® 10100 | 0.03 | 0.03 | 0.03 | 0.03 |
| Fatty amine (Ethomeen® C/12) | 0.3 | 0.3 | 0.5 | 0.4 |
| Fatty amide (Comperlan® LD 30) | 0.1 | 0.08 | 0.1 | 0.1 |

| | | | | |
|---|---|---|---|---|
| *Refers to a proprietary ATF additive package, Hitec© 403 but without Ethomeen T/12 (ex Ethyl Corp). | | | | |

The formulations in Tests 1-4 above passed the Electronically controlled converter clutch (ECCC) tests on the Mannesmann Sachs (MS) German for Geregelte Wandlerkupplung (hereafter "GWK"). The formulations shown above achieved a green shudder of 0 hours and a shudder resistance time of 110 hours or above (as against a specification time of a minimum of 100 hours) thereby meeting the demanding GWK requirements from MS and ZF.

## Claims

1. A friction modifier additive combination comprising
(a) an oil-soluble fatty amine compound of formula (I): wherein:
R is an alkyl group containing from 8 to 24 carbon atoms or any aryl group containing one or more alkyl substituents containing from 8 to 24 carbon atoms;
R¹ and R² are each independently an alkylene group containing from 1-8 carbon atoms; and x and y are each independently 0 or an integer from 1 to 5, and
(b) an oil-soluble fatty amide compound of the formula (II)
wherein R, R¹ and R², x and y are each independently as defined above for formula (I), and wherein the weight ratio of the fatty amine to fatty acid amide in the additive combination is in the range from 0.5:1 to 10:1.

2. A combination according to Claim 1, wherein the substituent groups R¹ and R² are each independently an alkylene group and have 1 to 4 carbon atoms.

3. A combination according to Claim 1 or 2, wherein the number of oxyalkylene groups represented by x and y are each independently suitably 0, 1 or 2 and are preferably 0.

4. A combination according to any one of Claims 1 to 3, wherein the fatty amine is selected from the group of coco-bis(2-hydroxyethyl)amine, a polyoxyethylene(5)coco-amine and an oleyl-bis- (2-hydroxyethyl)amine, and mixtures thereof.

5. A combination according to any one of Claims 1 to 4, comprising a mixture of (a) a bis(hydroxyethyl)fatty amine wherein the fatty group comprises an alkyl group which has 12 to 14 carbon atoms and (b) a bis (hydroxyethyl) fatty amide wherein the fatty group comprises an alkyl group which has 12 to 18 carbon atoms.

6. A lubricant formulation comprising a major amount of base oil of lubricating viscosity and a minor amount of a friction modifier additive combination as defined in any one of the preceding Claims 1-5.

7. A lubricant formulation according to Claim 6, wherein said formulation is an automatic transmission fluid having a kinematic viscosity at 100°C (KV ₁₀₀) ranging from 2-15 mm² /s measured according to the standard test procedure of ASTM D-446, a Brookfield viscosity at -40°C of less than 50,000 mPa s measured according to the standard test procedure of ASTM D-2983 and a viscosity index in the range from 100-200 measured according to the standard test procedure of ASTM D-2270.

8. A lubricant formulation according to Claim 6 or 7, wherein the total amount of the fatty amine and fatty acid amide present as the friction modifier additive combination is in the range from 0.05-1.2% by weight.

9. A lubricant formulation according to any one of the preceding Claims 6 to 8, wherein the base oil comprises a poly-alpha-olefin (PAO) having a KV₁₀₀ in the range from 2-8mm²/s.

10. A lubricant formulation according to any one of the preceding Claims 6 to 9, wherein said formulation comprises a mixture of a solvent refined mineral oil, a PAO and white oil.

11. A lubricant formulation according to any one of the preceding Claims 6 to 10, wherein said formulation comprises a viscosity index improver at a level of 2-15% by weight based on active ingredient.

12. A lubricant formulation according to Claim 11, wherein the viscosity index improver is a polymethylmethacrylate.

13. Use of the lubricant formulation according to any one of Claims 6 to 12 as a power transmission fluid.

14. Use of the lubricant formulation according to any one of Claims 6 to 12 as an automatic transmission fluid (ATF).

## Patentansprüche

1. Reibungsmodifizierer-Additivkombination, die
(a) öllösliche Fettaminverbindung mit der Formel (I): in der
R eine Alkylgruppe ist, die 8 bis 24 Kohlenstoffatome enthält, oder irgendeine Arylgruppe ist, die einen oder mehrere Alkylsubstituenten enthält, der/die 8 bis 24 Kohlenstoffatome enthält/enthalten:
R¹ und R² jeweils unabhängig eine Alkylengruppe sind, die 1 bis 8 Kohlenstoffatome enthält; und x und y jeweils unabhängig 0 oder eine Zahl von 1 bis 5 sind, und
(b) eine öllösliche Fettamidverbindung mit der Formel (II) umfasst, wobei R, R¹ und R², x und y jeweils unabhängig wie bereits für Formel (I) definiert sind, wobei das Gewichtsverhältnis des Fettamins zu dem Fettsäureamid in der Additivkombination im Bereich von 0,5:1 bis 10:1 liegt.

2. Kombination nach Anspruch 1, bei der die Substituentengruppen R¹ und R² jeweils unabhängig eine Alkylengruppe sind und 1 bis 4 Kohlenstoffatome aufweisen.

3. Kombination nach Anspruch 1 oder 2, bei der die Anzahl der durch x und y dargestellten Oxyalkylengruppen jeweils unabhängig geeigneterweise 0, 1 oder 2 ist und vorzugsweise 0 ist.

4. Kombination nach einem der Ansprüche 1 bis 3, bei der das Fettamin ausgewählt ist aus der Gruppe bestehend aus Kokos-bis(2-hydroxyethyl)amin, einem Polyoxyethylen(5)kokosamin und einem Oleyl-bis-(2-hydroxyethyl)amin und Mischungen derselben.

5. Kombination nach einem der Ansprüche 1 bis 4, die eine Mischung aus (a) Bis(hydroxyethyl)fettamin, bei dem die Fettgruppe eine Alkylgruppe umfasst, die 12 bis 14 Kohlenstoffatome enthält, und (b) Bis(hydroxyethyl)fettamid umfasst, bei dem die Fettgruppe eine Alkylgruppe umfasst, die 12 bis 18 Kohlenstoffatomen enthält.

6. Schmiermittelformulierung, die eine größere Menge Basisöl mit Schmierviskosität und eine kleinere Menge einer Reibungsmodifizierungs-Additivkombination, wie sie in einem der vorhergehenden Ansprüche 1 bis 5 definiert ist, umfasst.

7. Schmiermittelformulierung nach Anspruch 6, bei der die Formulierung ein Automatikgetriebefluid ist, das eine kinematische Viskosität bei 100°C (KV₁₀₀) im Bereich von 2 bis 15 mm²/s, gemessen nach dem Standardtestverfahren ASTM D-446, eine Brookfield-Viskosität bei -40°C von weniger als 50 000 mPa·s, gemessen nach dem Standardtestverfahren ASTM D-2983, und einen Viskositätsindex im Bereich von 100 bis 200, gemessen nach dem Standardtestverfahren ASTM D-2270, aufweist.

8. Schmiermittelformulierung nach Anspruch 6 oder 7, bei der die Gesamtmenge des Fettamins und Fettsäureamids, die in der Reibungsmodifizierer-Additivkombination vorhanden sind, im Bereich von 0,05 bis 1,2 Gew.-% liegt.

9. Schmiermittelformulierung nach einem der vorhergehenden Ansprüche 6 bis 8, bei der das Basisöl ein Poly-α-olefin (PAO) mit einer KV₁₀₀ im Bereich von 2 bis 8 mm²/s umfasst.

10. Schmiermittelformulierung nach einem der vorhergehenden Ansprüche 6 bis 9, bei der die Formulierung eine Mischung aus lösungsmittelraffiniertem Mineralöl, PAO und Weißöl umfasst.

11. Schmiermittelformulierung nach einem der vorhergehenden Ansprüche 6 bis 10, bei der die Formulierung einen Viskositätsindexverbesserer in einer Menge von 2 bis 15 Gew.-% umfasst, bezogen auf den wirksamen Bestandteil.

12. Schmiermittelformulierung nach Anspruch 11, bei der der viskositätsindexverbesserer ein Polymethylmethacrylat ist.

13. Verwendung der Schmiermittelformulierung gemäß einem der Ansprüche 6 bis 12 als Getriebefluid.

14. Verwendung der Schmiermittelformulierung gemäß einem der Ansprüche 6 bis 12 als Automatikgetriebefluid (ATF).

## Revendications

1. Combinaison d'additifs modifiant un frottement comprenant :
(a) un composé d'amine grasse soluble dans l'huile de formule (I) : dans laquelle :
R est un groupe alkyle contenant 8 à 24 atomes de carbone ou un groupe aryle quelconque contenant un ou plusieurs substituants alkyle contenant 8 à 24 atomes de carbone;
R¹ et R² sont chacun indépendamment un groupe alkylène contenant 1 à 8 atomes de carbone; et x et y sont chacun indépendamment 0 ou un entier de 1 à 5, et
(b) un composé d'amide gras soluble dans l'huile de formule (II) :
dans laquelle R, R¹ et R², x et y sont chacun indépendamment tels que définis ci-dessus pour la formule (I) et dans laquelle le rapport pondéral de l'amine grasse à l'amide d'acide gras de la combinaison d'additifs se situe dans la plage de 0,5:1 à 10:1.

2. Combinaison selon la revendication 1, dans laquelle les groupes substituants R¹ et R² sont chacun indépendamment un groupe alkylène et ont 1 à 4 atomes de carbone.

3. Combinaison selon la revendication 1 ou 2, dans laquelle le nombre de groupes oxyalkylène représentés par x et y est chacun indépendamment commodément de 0, 1 ou de 2, de préférence de 0.

4. Combinaison selon l'une quelconque des revendications 1 à 3, dans laquelle l'amine grasse est choisie dans le groupe constitué d'une coco-bis(2-hydroxyéthyl)amine, d'une polyoxyéthylène(5)cocoamine et d'une oléyl-bis-(2-hydroxyéthyl)amine et de leurs mélanges.

5. Combinaison selon l'une quelconque des revendications 1 à 4, comprenant un mélange (a) d'une bis(hydroxyéthyl)amine grasse, dans laquelle le groupe gras comprend un groupe alkyle qui a 12 à 14 atomes de carbone, et (b) d'un bis(hydroxyéthyl)amide gras, dans lequel le groupe gras comprend un groupe alkyle qui a 12 à 18 atomes de carbone.

6. Formulation de lubrifiant comprenant une quantité majeure d'huile de base de viscosité lubrifiante et une quantité mineure d'une combinaison d'additifs modificateurs de frottement comme défini dans l'une quelconque des revendications précédentes 1 à 5.

7. Formulation de lubrifiant selon la revendication 6, dans laquelle ladite formulation est un fluide de transmission automatique ayant une viscosité cinématique à 100°C (kV₁₀₀) dans la plage de 2 à 15 mm²/s, mesurée selon la procédure d'essai standard ASTM D-446, une viscosité Brookfield à -40°C de moins de 50 000 mPa.s, mesurée selon la procédure d'essai standard ASTM D-2983 et un indice de viscosité dans la plage de 100 à 200, mesuré selon la procédure d'essai standard ASTM D-2270.

8. Formulation de lubrifiant selon la revendication 6 ou 7, dans laquelle la quantité totale de l'amine grasse et de l'amide d'acide gras présents sous forme de combinaison d'additifs modificateurs de frottement se situe dans la plage de 0,05 à 1,2 % en poids.

9. Formulation de lubrifiant selon l'une quelconque des revendications précédentes 6 à 8, dans laquelle l'huile de base comprend une polyalphaoléfine (PAO) ayant un kV₁₀₀ dans la plage de 2 à 8 mm²/s.

10. Formulation de lubrifiant selon l'une quelconque des revendications précédentes 6 à 9, dans laquelle ladite formulation comprend un mélange d'une huile minérale raffinée au solvant, d'une PAO et d'une huile blanche (white oil).

11. Formulation de lubrifiant selon l'une quelconque des revendications 6 à 10, dans laquelle ladite formulation comprend un renforçateur d'indice de viscosité à un niveau de 2 à 15% en poids par rapport à l'ingrédient actif.

12. Formulation de lubrifiant selon la revendication 11, dans laquelle le renforçateur d'indice de viscosité est un poly(méthacrylate de méthyle).

13. Utilisation de la formulation de lubrifiant selon l'une quelconque des revendications 6 à 12 comme fluide de transmission d'énergie.

14. Utilisation de la formulation de lubrifiant selon l'une quelconque des revendications 6 à 12 comme fluide de boîte de vitesses automatique (ATF).
